# EUROPEAN PATENT SPECIFICATION

(11) **EP 2 574 439 B1**
(45) Date of publication and mention of the grant of the patent: **16.11.2016**
(21) Application number: 12185803.9
(22) Date of filing: 25.09.2012
(51) Int. Cl.: B29C 35/06, B29C 35/10, H01B 13/008, H01B 13/06, H01B 13/22, H01B 13/14, B05C 5/02, B05D 3/02

(54) **METHOD AND ARRANGEMENT OF CROSSLINKING OR VULCANISING AN ELONGATE ELEMENT**
VERFAHREN UND ANORDNUNG ZUR VERBINDUNG ODER VULKANISIERUNG EINES LÄNGLICHEN ELEMENTES
PROCÉDÉ ET AGENCEMENT POUR RÉTICULER OU VULCANISER UN ÉLÉMENT ALLONGÉ

(30) Priority: 30.09.2011 FI 20115960
(43) Date of publication of application: 03.04.2013
(73) Proprietor: Maillefer S.A., 1024 Ecublens (CH)
(72) Inventor: Karvonen, Esa, 90310 Oulu (FI)
(74) Representative: Kolster Oy Ab

(56) References cited:
- EP-A- 1 416 502
- EP-A1- 0 470 824
- CH-A5- 644 548
- GB-A- 1 592 958

## Description

The invention relates to a method of crosslinking or vulcanising an elongate element in which method a conductor element is coated by a layer of crosslinkable synthetic material in an extrusion step and the crosslinking reaction is carried out after the extrusion step and further in which method the conductor element is pre-heated in a pre-heating step before the extrusion step by generating inductively eddy currents inside the conductor element which will heat up the conductor element. The invention relates also to an arrangement for crosslinking or vulcanising an elongate element.

The present invention deals with a method and arrangement for inductive heating of electrical conductors used in the manufacturing of electrical wires and cables. It is directed at increasing the productivity of an electrical cable manufacturing line producing cables that have an insulation structure with at least one layer of crosslinked polyethylene, in particular medium and high voltage energy cables.

One widely used construction of energy transmission cables for medium and high voltage consist of an electrical conductor (Cu or Al), insulated with one or several layers of plastic material, very often polythylene. This insulation is applied onto the conductor in a per se known extrusion process. In order to provide sufficient mechanical and electrical strength, the extruded thermoplastic polymer material is crosslinked.

One method known in the prior art and widely used in the field for crosslinking is the peroxide crosslinking process. In this well-known process, peroxide is added to the thermoplastic material, which, under the effect of temperature, will eventually trigger the chemical reaction leading to the crosslinking of the polymer.

The principle layout of a vulcanising extrusion line is generally composed of a payoff, a metering capstan, a conductor preheater, an extrusion group with extrusion head, a postheater, a vulcanising tube, a cooling tube, a caterpillar or capstan and a take-up. Operation of such an extrusion line and its components are known per se and need not be discussed further. Note that in other line setups, the preheater can be placed upstream of the metering capstan.

In the manufacturing process described above, the insulation has to be extruded onto the conductor at a temperature sufficiently low as to avoid premature crosslinking in the extrusion equipment, as this would lead to defects of the insulation. After the extrusion step, the material has to be heated up at a temperature that is sufficiently high to start and complete the chemical reaction within the shortest possible time.

The crosslinking reaction is carried out in the vulcanisation tube, i.e. a tube surrounding the extruded electrical cable located downstream of the extrusion head, inside which the cable is heated up by radiant and/or convective heat transfer. The heat diffusion in the insulation is however low, and the polymer layers close to the conductor element will take the longest time to increase temperature and undergo the chemical reaction.

A method known in the prior art to improve this heating/crosslinking process is to pre-heat the conductor prior to the extrusion step. This preheating is obtained by means of inductively generating eddy currents inside the conductor element which will heat up the conductor element. Therefore, heat is transferred into the insulation structure from inside the cable, and the heating/crosslinking process completes in shorter time. Such inductive heating elements have been known and used for a long time. Said inductive heating elements are used as pre-heaters upstream of the extrusion head and as post-heaters downstream of the extrusion head and along the vulcanisation tube. As an example of the arrangements discussed above CH Patent No. 644 548 can be mentioned.

Another example is EP 0 470 824 A1 which describes pre-heating of the core of a cable. The amount of preheating and the beneficial effect on productivity is however limited with the known arrangements for the following reason. In most energy cable constructions, the conductors are stranded wires consisting of multiple layers of wires. Preheaters used for conductor preheating use frequencies in the range of 7-20 kHz. The penetration depth of the magnetic field created by said preheaters into the conductor is limited. Especially in conductors with large cross-sections, the preheaters used heat up only the outermost layers of stranded wires of the conductor. Owing to said fact the temperature of outermost layer rises quickly, while the temperature rises with a certain delay at the core of the conductor. At the exit of the preheater, temperatures between outermost and innermost layers differ by a certain amount DT. The value of this difference DT depends on the intensity of the eddy currents and the duration of exposure of the conductor to the electrical field, i.e. the length of the preheater divided by the line speed. Downstream of the preheater, the temperature would substantially equalize over the cross-section of the conductor to an average temperature Tm within a certain time, depending on the size of the conductor and the temperature difference DT.

If the temperature difference DT gets large enough, differential thermal expansion between the outermost and inner layers will lead to loss of contact between layers and eventually to opening up of the conductor. As a consequence not only the heat is no longer transferred to the inner layers of wires of the conductor, but plastic material may penetrate between the outermost wires. In extreme cases, thermal expansion may be such that the conductor gets stuck in the wire-guide in the extrusion head.

Owing to the facts above, the rate of pre-heating that can be applied to the conductor, and as a consequence the conductor temperature obtained, is limited.

The matters discussed above are problems of the prior art. The object of the invention is to obtain a method and an arrangement by which the problems of the prior art can be solved. This is obtained with the invention. The method of the invention is characterized in that the pre-heating step is carried out by increasing temperature of the conductor element gradually so that temperature difference between outermost region of the conductor element and the inner layer of the conductor element remains below a pre-determined level at the end of the pre-heating step. The arrangement of the invention is characterized in that the device carrying out pre-heating is arranged to increase temperature of the conductor element gradually so that temperature difference between outermost region of the conductor element and the inner layer of the conductor element remains below a pre-determined level at the exit of the device carrying out pre-heating.

An advantage of the invention is in that is solves the problems of the prior art discussed above. In other words the invention offers a method and an arrangement by which it is possible to increase the conductor temperature prior to the extrusion step to higher levels than previously possible, in order to boost production speed of the extrusion line.

In the following the invention will be described in greater detail with reference to embodiments shown in the attached drawing, whereby
Figure 1 shows a principle layout of a vulcanising extrusion line,
Figure 2 shows a schematical cross section of a conductor element,
Figure 3 shows a schematical temperature profile in a conductor element along a typical prior art pre-heater,
Figure 4 shows a schematical temperature profile in a conductor element along an embodiment of the pre-heater of the present invention and compared to the typical prior art solution and
Figure 5 shows a schematical temperature profile in a conductor element along another embodiment of the pre-heater of the present invention.

Figure 1 shows a principle layout of a vulcanizing extrusion line. The vulcanising extrusion line comprised a payoff 1, a metering capstan or metering caterpillar 2, a preheater 3 for a conductor element, as extrusion group with an extrusion head 4, a postheater 5, a vulcanising tube 6, a cooling tube 7, a caterpillar or a capstan 8 and a take-up 9. As said earlier operation of the extrusion line described above is well-known to a person skilled in the art, and therefore operation or/and construction of the extrusion line is not described in detail here.

Figure 2 shows schematically a typical conductor element consisting stranded wires 10. As shown in Figure 2 the conductor element comprises multiple layers of wires 10. In Figure 2 reference a shows the outermost region or layer of the conductor element and reference b shows the inner layer, i.e. the core layer of the conductor element.

As told earlier it has been known for long that insulation layer has been applied onto the conductor element by using an extruder. Said insulation layer consisting for example of thermoplastic polymer material, has been applied onto the conductor and crosslinked. Said crosslinking has been carried out by using a peroxide crosslinking process in which the effect of temperature triggers the chemical reaction leading to the crosslinking of the polymer. The crosslinking reaction has been carried out in the vulcanising tube 6. The heat diffusion in the insulation layer is however low, and therefore the polymer material close to the conductor element takes rather long time to increase temperature and undergo the chemical reaction when compared to the outermost layer of the polymer material of the insulation layer. In order to improve the situation it has been known in the field to improve the crosslinking process by pre-heating the conductor element prior to the extrusion step. Said pre-heating has been carried out inductively, i.e. by generating eddy currents inside the conductor element which heats up the conductor element. This means in practice that heat is transferred into the insulation layer extruded also from inside, and therefore said crosslinking process is speeded up.

Figure 3 shows a schematical temperature profile in a conductor element along a typical prior art pre-heater. As shown in Figure 3 the temperature of the outermost layer a rises rather quickly. The temperature in the inner layer b rises clearly slowly when compared to the temperature of the outermost layer a. At the exit of the pre-heater temperatures between the outermost layer and the inner layer differ by a certain amount shown by the reference DT in Figure 3.

As discussed above the value of the difference DT depends on the intensity of the eddy currents and the duration of exposure of the conductor element to the electrical field. Downstream of the pre-heater, the temperature substantially equalizes over the cross-section of the conductor element to an average temperature Tm within a certain time, depending on the size of the conductor element and the temperature difference DT.

It must be noted here that if the temperature difference DT gets large enough, differential thermal expansion between the outermost layer and the inner layer leads easily to loss of contact between said layers and eventually to opening up of the wires of the conductor element. As a consequence not only the heat is no longer transferred to the inner layers of wires of the conductor element, but plastic material may penetrate between the wires of the outermost layer. In extreme cases, thermal expansion may be such that the conductor element gets stuck in the wire-guide in the extrusion head. The problem described above is pretty severe especially with aluminium conductors due to oxidized surface of wires, and also in wires covered with lacquer.

The matters described above mean that the rate of pre-heating that can be applied to the conductor element, and as a consequence the conductor temperature obtained, is limited.

Figure 4 shows schematically the basic principle of the invention when compared to the prior art. The prior art is shown by describing how the temperatures rise in a short pre-heater. This part of Figure 4 corresponds to Figure 3. The temperature difference between the outermost layer a and the inner layer b of the conductor part at the exit of said short pre-heater is shown with a reference DTs. Average temperature after said short pre-heater is shown with a reference Tms in Figure 4. According to the basic idea of the invention the pre-heating step is carried out by increasing temperature of the conductor element slower, i.e. gradually so that temperature difference between outermost layer or region a of the conductor element and the inner layer b of the conductor element remains below a pre-determined level at the end of the pre-heating step. In other words with the invention it is possible to obtain essentially the same average temperature as obtained with the prior art but with clearly smaller temperature difference DTI at the exit of the pre-heater. It is also possible with the invention to obtain higher line speeds that by using the prior art. This is because the temperature difference at the exit of the preheater can always in all operating conditions can be kept below a certain pre-determined level This means that the disadvantages of the prior art described above can be eliminated.

In the embodiment of Figure 4 a long pre-heater is used, and the effect of the long coil, i.e. a long pre-heater is shown with dotted lines in figure 4. The temperature difference at the exit of the long pre-heater is shown with a reference DTI in Figure 4. Average temperature after said long pre-heater is shown with a reference Tml in Figure 4. Figure 4 shows clearly that DTI is smaller than DTs.

Due to the longer exposure, the induced power can be reduced and therefore the temperature difference between the outermost layer a and the inner layer b of the conductor element is reduced to an acceptable level. The length of the pre-heater can be dimensioned so that a certain pre-determined level is reached for DTI.

Figure 4 shows basically an embodiment of the invention in which longer exposure with reduced power is carried out in one continuous step. This is however not the only possibility but it is possible to materialize the basic idea of the invention also in other ways.

Figure 5 refers schematically to an embodiment in which the heating step is carried out with two successive steps, i.e. by using a pre-heater 1 and a pre-heater 2. In the embodiment of Figure 5 said two pre-heaters, i.e. induction coils, are placed at intervals so that the temperature inside the conductor element evolves in a way that the temperature difference between the outermost layer and the inner layer does not lead to excessive thermal expansion differences between the wires of the conductor element. The temperature differences at the exits of the pre-heaters are shown with references DT1 and DT2 in Figure 5.

In the embodiment of Figure 5 the two pre-heaters are placed at a distance to each other. Induction power is maintained at a level so that no detrimental expansion occurs at the exits of the pre-heaters. The distance of the first pre-heater to the second pre-heater is determined so that the temperature in the conductor element becomes uniform across the conductor element before the conductor element enters the second pre-heater. Said uniform temperature, i.e. the average temperature after the first pre-heater, is shown with reference Tm1 in Figure 5. In the second pre-heater, the average conductor element temperature is raised to a substantially higher level without damaging the conductor element. The average temperature after the second pre-heater is shown with reference Tm1+2 in Figure 5.

The embodiment of Figure 5 uses two pre-heaters. It is however quite possible to use more than two pre-heaters placed with pre-determined distances to each other in the way as described above in connection with the embodiment of Figure 5.

When for example two step pre-heating is used it is possible that the first pre-heater is located before the metering capstan or metering caterpillar, i.e. the step shown with reference number 2 in Figure 1. It is however also possible to locate both pre-heaters after the metering capstan or metering caterpillar, i.e. the step shown with reference number 2 in Figure 1.

It is also quite possible within the spirit of the invention to use for example two pre-heaters arranged contiguously to each other. This embodiment is advantageous for example in creating a long pre-heater in order to obtain a long and continuous pre-heating step.

The optimum distance between separate successive pre-heaters depends on the pre-heater used and also on production conditions. It is quite possible to make the pre-heaters as a movable construction in order to enable finding of the optimum distance in various production conditions.

The constructions shown are not the only possibilities to materialize the invention but, the constructions may be for example such that pre-heaters or at least one of them can be taken away and arranged to a different position. Alternatively the pre-heaters or at least one of them may be mounted to a movable platform construction. Said movable platform construction may enable either stepwise movement or continuous movement or even both.

The present invention can be supported by using the following data obtained from the field test.
Line: CCV, 10 x 6 m heating, 145 m water cooling
   1. Al 150 mm2 20kV (0,7 mm + 5,5 mm + 0,6 mm):
      - T(preheat) 20... 110 deg C → v=19,6 m/min
      - T(preheat1) 20...80 deg C + T(preheat2) 80...145 deg C →24,4 m/min
   2. Al 150 mm2 10 kV (0,7 mm + 3,4 mm + 0,6 mm):
      - T(preheat) 20...110 deg C → 31,2 m/min
      - T(preheat1) 20...80 deg C + T(preheat2) 80...145 deg C → v= 40,0 m/min

The examples shown above prove that by using gradual heating, in these cases stepwise materialized heating step, it is possible to obtain higher line speeds. In other words the invention is clearly beneficial for productivity.

## Claims

1. Method of crosslinking or vulcanising an elongate element in which method a conductor element is coated by a layer of crosslinkable synthetic material in an extrusion step (4) and the crosslinking reaction is carried out after the extrusion step (4) and further in which method the conductor element is pre-heated in a pre-heating step (3) before the extrusion step by generating inductively eddy currents inside the conductor element which will heat up the conductor element, **characterized in that** the pre-heating step (3) is carried out by increasing temperature of the conductor element gradually so that temperature difference (DT) between outermost region (a) of the conductor element and the inner layer (b) of the conductor element remains below a pre-determined level at the end of the pre-heating step.

2. Method as claimed in claim 1, **characterized in that** the pre-heating step (3) is carried out in one continuous step.

3. Method as claimed in claim 1, **characterized in that** the pre-heating step (3) is carried out with at least two successive steps.

4. Method as claimed in claim 3, **characterized in that** there is a distance between the two successive steps and the distance is determined so that after one step the temperature becomes uniform across the conductor element before another step is carried out.

5. Arrangement for crosslinking or vulcanising an elongate element in which arrangement a conductor element is coated by a layer of crosslinkable synthetic material by using an extrusion head (4) and the crosslinking reaction is carried out after the extrusion (4) head in a vulcanization tube and further in which arrangement the conductor element is pre-heated before the extrusion head by a device (3) arranged to generate inductively eddy currents inside the conductor element which will heat up the conductor element, **characteriz ed** in that in that the device (3) carrying out pre-heating is arranged to increase temperature of the conductor element gradually so that temperature difference (DT) between outermost region (a) of the conductor element and the inner layer (b) of the conductor element remains below a pre-determined level at the exit of the device (3) carrying out pre-heating.

6. Arrangement as claimed in claim 5, **characterized in that** a device (3) inductively creating eddy currents is formed by one induction coil.

7. Arrangement as claimed in claim 5, **characterized in that** a device (3) inductively creating eddy currents is formed by at least two successively arranged induction coils.

8. Arrangement as claimed in claim 7, **characterized in that** there is a distance between the two successive induction coils and the distance between the two successive induction coils is determined so that after one induction coil the temperature (Tm) becomes uniform across the conductor element before another induction coil.

9. Arrangement as claimed in claim 7, **characterized in that** the two successive induction coils have been arranged contiguously to each other.

10. Arrangement as claimed in any of the claims 7 - 9, **characte rized** in that at least one the induction coils is formed as a movable construction.

## Patentansprüche

1. Verfahren zum Vernetzen oder Vulkanisieren eines länglichen Elementes, wobei in diesem Verfahren ein Leiterelement durch eine Schicht aus vernetzbarem, synthetischem Material in einem Extrusionsschritt (4) beschichtet wird und die Vernetzungsreaktion nach dem Extrusionsschritt (4) durchgeführt wird und des Weiteren in diesem Verfahren das Leiterelement in einem Vorheizschritt (3) vor dem Extrusionsschritt durch induktives Erzeugen von Wirbelströmen, die das Leiterelement aufheizen, innerhalb des Leiterelementes vorgewärmt wird, **dadurch gekennzeichnet, dass** der Vorheizschritt (3) durch allmähliches Erhöhen der Temperatur des Leiterelements durchgeführt wird, so dass die Temperaturdifferenz (DT) zwischen dem äußersten Bereich (a) des Leiterelementes und der inneren Schicht (b) des Leiterelementes unter einem vorbestimmten Niveau am Ende des Vorheizschrittes bleibt.

2. Verfahren nach Anspruch 1, **dadurch gekennzeichnet, dass** der Vorheizschritt (3) in einem durchgehenden Schritt durchgeführt wird.

3. Verfahren nach Anspruch 1, **dadurch gekennzeichnet, dass** der Vorheizschritt (3) mit wenigstens zwei aufeinanderfolgenden Schritten durchgeführt wird.

4. Verfahren nach Anspruch 3, **dadurch gekennzeichnet, dass** es einen Abstand zwischen den zwei aufeinanderfolgenden Schritten gibt und der Abstand so bestimmt wird, dass nach einem Schritt die Temperatur gleichmäßig über das Leiterelement verteilt ist, bevor ein weiterer Schritt durchgeführt wird.

5. Anordnung zum Vernetzen oder Vulkanisieren eines länglichen Elementes, wobei in dieser Anordnung ein Leiterelement mit einer Schicht aus vernetzbarem Kunststoffmaterial unter Verwendung eines Extrusionskopfes (4) beschichtet wird und die Vernetzungsreaktion nach dem Extrusionkopf (4) in einem Vulkanisationsrohr durchgeführt wird und wobei des Weiteren in dieser Anordnung das Leiterelement vor dem Extrusionskopf durch eine Vorrichtung (3) vorgeheizt wird, die angeordnet ist, um induktiv Wirbelströme, die das Leiterelement aufheizen, innerhalb des Leiterelements zu erzeugen, **dadurch gekennzeichnet, dass** die Vorrichtung (3), welche das Vorheizen durchführt, so angeordnet ist, um die Temperatur des Leiterelementes allmählich zu erhöhen, so dass der Temperaturunterschied (DT) zwischen dem äußersten Bereich (a) des Leiterelementes und der inneren Schicht (b) des Leiterelementes am Ausgang der Vorrichtung (3), welche das Vorheizen durchführt, unter einem vorbestimmten Pegel bleibt.

6. Anordnung nach Anspruch 5, **dadurch gekennzeichnet, dass** eine Vorrichtung (3), welche induktiv Wirbelströme erzeugt, durch eine Induktionsspule gebildet ist.

7. Anordnung nach Anspruch 5, **dadurch gekennzeichnet, dass** eine Vorrichtung (3), welche induktiv Wirbelströme erzeugt, durch mindestens zwei nacheinander angeordnete Induktionsspulen gebildet ist.

8. Anordnung nach Anspruch 7, **dadurch gekennzeichnet, dass** ein Abstand zwischen den zwei aufeinanderfolgenden Induktionsspulen besteht und der Abstand zwischen den zwei aufeinanderfolgenden Induktionsspulen bestimmt ist, so dass nach einer Induktionsspule die Temperatur (Tm) gleichförmig über das Leiterelement vor einer weiteren Induktionsspule ist.

9. Anordnung nach Anspruch 7, **dadurch gekennzeichnet, dass** die beiden aufeinanderfolgenden Induktionsspulen aneinander angrenzend zueinander angeordnet sind.

10. Anordnung nach einem der Ansprüche 7 - 9, **dadurch gekennzeichnet, dass** zumindest eine der Induktionsspulen als ein beweglicher Aufbau ausgebildet ist.

## Revendications

1. Méthode de réticulation ou de vulcanisation d'un élément allongé, méthode dans laquelle un élément conducteur est revêtu d'une couche de matériau synthétique réticulable dans une étape d'extrusion (4) et la réaction de réticulation est réalisée après l'étape d'extrusion (4) et méthode dans laquelle en outre l'élément conducteur est préchauffé dans une étape de préchauffage (3) avant l'étape d'extrusion en générant inductivement des courants de Foucault à l'intérieur de l'élément conducteur ce qui réchauffera l'élément conducteur, **caractérisée en ce que** l'étape de préchauffage (3) est réalisée en augmentant la température de l'élément conducteur graduellement de telle sorte que la différence de température (DT) entre la région le plus à l'extérieur (a) de l'élément conducteur et la couche interne (b) de l'élément conducteur reste en dessous d'un niveau prédéterminé à la fin de l'étape de préchauffage.

2. Méthode selon la revendication 1, **caractérisée en ce que** l'étape de préchauffage (3) est réalisée dans une étape continue.

3. Méthode selon la revendication 1, **caractérisée en ce que** l'étape de préchauffage (3) est réalisée en au moins deux étapes successives.

4. Méthode selon la revendication 3, **caractérisée en ce qu'**il existe une distance entre les deux étapes successives et la distance est déterminée de telle sorte qu'après une étape, la température devient uniforme au travers de l'élément conducteur avant qu'une autre étape ne soit réalisée.

5. Agencement pour réticuler ou vulcaniser un élément allongé, agencement dans lequel un élément conducteur est revêtu d'une couche de matériau synthétique réticulable à l'aide d'une tête d'extrusion (4) et la réaction de réticulation est réalisée après la tête d'extrusion (4) dans un tube de vulcanisation et agencement dans lequel en outre l'élément conducteur est préchauffé avant la tête d'extrusion à l'aide d'un dispositif (3) agencé pour générer inductivement des courants de Foucault à l'intérieur de l'élément conducteur ce qui réchauffera l'élément conducteur, **caractérisée en ce que** le dispositif (3) réalisant le préchauffage est agencé pour accroître la température de l'élément conducteur graduellement de telle sorte que la différence de température (DT) entre la région le plus à l'extérieur (a) de l'élément conducteur et la couche interne (b) de l'élément conducteur reste en dessous d'un niveau prédéterminé à la sortie du dispositif (3) réalisant le préchauffage.

6. Agencement selon la revendication 5, **caractérisé en ce qu'**un dispositif (3) créant inductivement des courants de Foucault est formé par une bobine d'induction.

7. Agencement selon la revendication 5, **caractérisé en ce qu'**un dispositif (3) créant inductivement des courants de Foucault est formé par au moins deux bobines d'induction agencées successivement.

8. Agencement selon la revendication 7, **caractérisé en ce qu'**il existe une distance entre les deux bobines d'induction successives et la distance entre les deux bobines d'induction successives est déterminée de telle sorte qu'après une bobine d'induction, la température (Tm) devient uniforme au travers de l'élément conducteur avant une autre bobine d'induction.

9. Agencement selon la revendication 7, **caractérisé en ce que** les deux bobines d'induction successives ont été agencées de manière contiguë l'une par rapport à l'autre.

10. Agencement selon l'une quelconque des revendications 7 à 9, **caractérisé en ce qu'**au moins l'une des bobines d'induction se présente sous la forme d'une construction mobile.
